

## UNITED STATES PATENT OFFICE.

JAMES ELIOT BOOGE, OF NEWARK, AND MARION L. HANAHAN, OF EAST ORANGE, NEW JERSEY, ASSIGNEES, BY MESNE ASSIGNMENTS, TO THE GRASSELLI CHEMICAL COMPANY, OF CLEVELAND, OHIO, A CORPORATION OF DELAWARE.

## LITHOPONE COMPOSITION AND PROCESS OF MAKING SAME.

No Drawing.

Application filed February 11, 1928. Serial No. 253,782.

This invention relates to the production of a lithopone pigment having improved mixing and dispersing properties in paint vehicles, and more particularly to lithopone treated with a water soluble soap under conditions to allow uniform adsorption upon the surface of pigment particles.

This case is a continuation in part of our application Serial No. 742,423, filed Oct. 8, 10 1924.

Lithopone is a white pigment very widely used in the paint industry. It is composed of approximately 29% zinc sulfide and 71% barium sulfate. These compounds are 15 precipitated from solutions of barium sulfate and zinc sulfate, the precipitate is then dried, calcined, quenched, ground to a fine state of division, filtered, dried, and disintegrated.

20 The use of sodium and potassium silicate has been suggested (French patent to Gademann, 407,642 of 1909) as added agents to help make lithopone light stable, but these materials have not proved satisfactory for 25 producing a light stable product. Lithopone treated with sodium silicate does not show improved mixing and dispersion in paint vehicles.

The use of oil-soluble soaps in paints has 30 also been suggested (British patent to Allendorff, 23,687 of 1906), but they have been introduced merely to thicken the paint and give a false body, and do not function as dispersing agents in the sense of facilitating mixing 35 of the pigment with the vehicle. Although Allendorff states that the use of oil-soluble soap renders the lithopone light resistant, this has proved an inoperative conception.

Very rapid progress has been made during 40 the last few years in the improvement of the lithopone process. Light resistant pigments have been developed which are also very much superior in color and hiding power as compared with the lithopone of several years ago. 45 The production of a light resistant lithopone, however, involves one disadvantage. The ease of mixing with paint vehicles is adversely affected. The older light sensitive type of lithopone had a reputation of being 50 rather tricky in paint formulas. It had a tendency to "fight the oil." By this expression the paint man meant difficult mixing or wetting by the vehicle. This tendency is in-

creased in the light resistant lithopone made 55 according to the more recent prior art.

The ordinary paint mixing operation is carried out in vertical cylindrical iron mixers with a capacity of 50-100 gals. They are fitted with vertical rotating paddles which 60 cut through and mix the mass of pigment and vehicle. The vehicle is introduced first, and then the proper amount of lithopone is added. Poor mixing lithopone will set up with the vehicle to form a more or less plastic sticky 65 mass. In extreme cases the mixture assumes a stiff putty-like consistency which may even break the mixer blades, twist the driving shaft, etc. Ordinarily, however, the disadvantage lies in the extra power consumption 70 and the greatly decreased capacity of the equipment due to the longer mixing period required. The latter is a particularly serious disadvantage and precludes the use of poor mixing lithopone in many formulas. 75

An object of this invention is to overcome the poor wetting and dispersing properties of lithopone in paint. A further object is the production of a coating on the pigment particles with affinity for the organic liquids in 80 the paint vehicle. Other objects will appear as the description proceeds.

These objects are accomplished by treatment of the lithopone in the form of a water slurry with a solution of a soap. The treatment is made in such manner that each pigment particle comes into contact with the soluble soap and has an opportunity to adsorb a protective film of the latter. The lithopone is treated at some point following the calcination and prior to the final drying. This is done so that the lithopone may be in the form 90 of a water slurry where the particles are essentially separated and free to adsorb a film of soap from the solution of the latter. Further, the reaction of the lithopone slurry must be neutral or alkaline to avoid the decomposition of the soap with liberation of the insoluble fatty acids.

We have found that water soluble soaps, 100 such as rosin soaps, and the usual water-soluble washing soaps, such as Ivory, and para soaps, the latter being the soap of sulfonated castor oil, are very effective dispersing agents for lithopone and produce a greatly improved 105 light stable product. This water solubility of these soaps is highly important as it provides

for adding the soap to the water slurry so that the soap will be present during the filter-pressing and drying to resist any tendency of the particles to aggregate and cement together.

In our preferred process we treat the lithopone slurry just prior to the final filtration and drying. This slurry contains approximately 2 parts of water to one part of pigment.

10 It is contained in a tank equipped with efficient agitating means so that the whole mass of slurry is turned over and mixed rapidly and continuously. The soap solution is run into this tank, preferably at the bottom 15 and immediately mixes with the agitated slurry. The solution used should be relatively low in concentration, say 1-4% and the temperature should be below the boiling point. The amount of soap added will vary 20 with the degree of dispersion desired in the finished product. In general 1% is sufficient to give a definite effect, .5% is usually sufficient for perfect mixing and dispersion but greater quantities may be desirable in special 25 cases. These percentages are for dry weight of soap based upon actual pigment content.

The following examples are given by way of illustration but it will be understood that these are not to be taken as in any way limiting 30 our invention.

#### Example I.

Lithopone slurry containing two parts of water to one of pigment is introduced into a 35 wooden tank 12 ft. in diameter and 12 ft. deep. This tank is furnished with a high speed turbine agitator, giving rapid mixing of the slurry. There are present 12 tons of dry lithopone and 24 tons of water. The reaction 40 of the slurry is neutral with a pH of 7.0. In a separate smaller tub an amount of "para soap" corresponding to .5% based upon the lithopone, dry weight, is dissolved in water. The para soap is sulphonated castor oil 45 neutralized with ammonium hydroxide. It contains 60% of total fats. The soap is dissolved in sufficient water at 70° C. to give a 4% solution. This solution is pumped into the bottom of the lithopone slurry tank 50 throughout a period of 6 hours. The agitation is continued during the addition of the soap and 1 hour thereafter. At the end of this period the batch is filter pressed, dried and disintegrated in the usual manner.

#### Example II.

Lithopone slurry is introduced into the same tank described under Example No. I and in similar concentration and quantity. The 60 soap used in this case is the sodium salt of oleic acid. The soap solution is made up in a separate tank from sodium carbonate and commercial oleic acid known as Red oil. An amount of oleic acid equivalent to 1% based 65 upon the lithopone is used. A sodium car-

bonate solution is first made up with an amount of soda ash equivalent to the oleic acid. This solution is heated to 60° C. and the oleic acid slowly added with efficient agitation. When saponification is completed the 70 soap solution is pumped into the lithopone slurry in the same manner described under Example No. I and the lithopone is finished as described there.

#### Example III.

This treatment is made in the same manner as that made under Example No. I except that 2% of a commercial washing soap is used. The soap is obtained in chip form and consists essentially of sodium stearate with some oleate. An amount of soap equal to 2% of the lithopone dry weight is weighted up and dissolved at a temperature somewhat below the boiling point. The concentration of the solution is 4%. It is added to the lithopone slurry in the same manner as described under Example No. I and lithopone is then finished in the same way.

In the above examples three types of soap 90 have been cited. In addition to these we may use any other water soluble soap including the ammonium, sodium, potassium, etc., salts of the fatty acids, of the sulfonated fats and fatty acids and of rosin. Insoluble soaps are 95 not satisfactory presumably due to the lack of proper distribution on the lithopone particles.

The theory of the action of these soaps has 100 already been referred to briefly. It is believed that the soap is adsorbed upon the surface of the lithopone particles to produce a more or less continuous film. This adsorption occurs with the carboxyl end or the acid group pointed inward toward the pigment 105 particle. This allows the hydrocarbon or "non-polar" end of the molecule to point outward. As a result the film around the particle is of such type that it attracts or has an affinity for the organic liquids in the paint vehicle. This leads to easy and complete 110 wetting of the individual particles by the paint vehicle.

Further, as a result of the complete wetting 115 there is perfect dispersion of the pigment in the paint. In other words all the pigment particles are separate from each other and not bound together in flocculates or groups. This results in improved properties of the paints such as increased flow, better gloss and hiding power. These paint properties conferred by complete dispersion are of definite importance to the paint manufacturer.

One method for determining the wetting and dispersing properties of lithopone is by 125 use of mineral thinner. It is well known that mineral thinner or turpentine substitute is one of the poorest dispersing constituents of paint vehicles. When the ordinary lithopone is added to mineral thinner, the wetting 130

is very poor and the mixture forms a solid flocculated mass. A relatively high amount of thinner is required to reduce the mixture to a consistency approaching that of paint 5 and even so, it has no flow or brushing properties. With the lithopone produced as described in Example No. I even mineral thinner will wet the pigment to give a paint like mixture.

10 The test may be carried out by the use of 5 grams of lithopone and addition thereto of 1.5 c. c. of mineral thinner. The mixture is then rubbed down under a spatula and a paint like product results. The ordinary lithopone 15 of the prior art subjected to this test gives a mass which is almost dry and at least 5 c. c. of the mineral thinner are required to break it down,—even, so the mixture shows no paint like flow or brushing properties.

20 As many apparently widely different embodiments of this invention may be made without departing from the spirit therof, it is to be understood that we do not intend to limit ourselves to the specific embodiments 25 thereof except as indicated in the appended claims.

We claim:

1. The process of improving the mixing and dispersing properties of lithopone pigment in paint vehicles which comprises treating the lithopone with a water-soluble soap. 30 2. The process of improving the mixing and dispersing properties of lithopone pigment in paint vehicles which comprises treating the lithopone with water-soluble soap in an amount varying from .1% to 2%. 35 3. The process of improving the mixing and dispersing properties of lithopone pigment in paint vehicles which comprises treat-

ing the lithopone with ammonium soap.

4. The process of improving the mixing and dispersing properties of lithopone pigment in paint vehicles which comprises treating the lithopone with para soap. 40

5. A lithopone composition of improved 45 paint mixing properties comprising light resistant lithopone and a water-soluble soap.

6. A lithopone composition of improved paint mixing properties comprising light resistant lithopone and water-soluble soap in an 50 amount varying from .1% to 2%.

7. A lithopone composition of improved paint mixing properties comprising light resistant lithopone and ammonium soap.

8. A lithopone composition of improved 55 paint mixing properties comprising light resistant lithopone and para soap.

9. A lithopone water-soluble soap composition capable of producing a paint like mixture when 5 grams of said composition are mixed 60 with approximately 1.5 c. c. of a mineral thinner.

10. The process of improving the paint mixing properties of light-resistant lithopone which comprises mixing a water-soluble dispersing agent comprising a soap with the light-resistant lithopone after the calcination and quenching, and prior to drying 65 therof.

11. A calcined lithopone pigment composition of improved paint-mixing properties comprising light-resistant lithopone and a water-soluble dispersing agent comprising a soap adhering to the pigment particles. 70

In testimony whereof we affix our signatures.

JAMES ELIOT BOOGE.  
MARION L. HANAHAN.